# EUROPEAN PATENT SPECIFICATION

(11) **EP 0 177 669 B1**
(45) Date of publication and mention of the grant of the patent: **04.03.1992**
(21) Application number: 85105338.9
(22) Date of filing: 02.05.1985
(51) Int. Cl.: C22C 38/00, H01F 1/16

(54) **Amorphous metal alloys having enhanced AC magnetic properties at elevated temperatures**
Amorphe Metallegierungen mit magnetischen Eigenschaften in Wechselstrom bei hohen Temperaturen
Alliages métalliques amorphes présentant des propriétés magnétiques en courant alternatif aux températures élevées

(30) Priority: 23.05.1984 US 613118; 16.08.1984 US 641145
(43) Date of publication of application: 16.04.1986
(73) Proprietor: AlliedSignal Inc., Morristown New Jersey 07962-2245 (US)
(72) Inventor: Nathasingh, Davidson M., Morristown, NJ 07960 (US); Martis, Ronald Joseph Jacob, Morristown, NJ 07960 (US); Datta, Amitava, Morristown, NJ 07960 (US)
(74) Representative: Weber, Dieter, Dr.

(56) References cited:
- EP-A- 0 058 269
- EP-A- 0 060 660
- EP-A- 0 095 831
- US-A- 4 217 135

## Description

The invention relates to amorphous metal alloy compositions and, in particular, to amorphous alloys containing iron, silicon and boron hvaing enhanced AC magnetic properties at elevated temperatures.

Investigations have demonstrated that it is possible to obtain solid amorphous materials from certain metal alloy compositions. An amorphous material substantially lacks any long range atomic order and is characterized by an X-ray diffraction profile consisting of broad intensity maxima. Such a profile is qualitatively similar to the diffractioin profile of a liquid or ordinary window glass. This is in contrast to a crystalline material which produces a diffraction profile consisting of sharp, narrow intensity maxima.

These amorphous materials exist in a metastable state. Upon heating to a sufficiently high temperature, they crystallize with evolution of the heat of crystallization, and the X-ray diffraction profile changes from one having amorphous characteristics to one having crystalline characteristics.

Novel amorphous metal alloys have been disclosed in US-A- 3 856 513
These amorphous alloys have the formula MₐY_{b}Z_{c} where M is at least one metal selected from the group of iron, nickel, cobalt, chromium and vanadium, Y is at least one element selected from the group consisting of phosphorus, boron and carbon, Z is at least one element selected from the group consisting of aluminum, antimony, beryllium, germanium, indium, tin and silicon, "a" ranges from about 60 to 90 atom percent, "b" ranges from about 10 to 30 atom percent and "c" ranges from about 0.1 to 15 atom percent. These amorphous alloys have been found suitable for a wide variety of applications in the form of ribbon, sheet, wire, powder, etc. The US-A-3 856 513 also discloses amorphous alloys having the formula TᵢXⱼ , where T is at least one transition metal, X is at least one element selected from the group consisting of aluminum, antimony, beryllium, boron, germanium, carbon, indium, phosphorus, silicon and tin, "i" ranges from about 70 to 87 atom percent and "j" ranges from about 13 to 30 atom percent. These amorphous alloys have been found suitable for wire applications.

US-A- 4 300 950 discloses amorphous metal alloys consisting essentially of 12 to 15% boron, 1 to 8% silicon and 80 to 84% iron, by atomic percentage. These alloys exhibit relatively low crystallization and curie temperatures (i.e. less than 400°C). As a result, the magnetic properties thereof are substantially degraded by long term thermal aging, and the induction levels of the alloys are relatively low at elevated temperatures. Hence, the alloys are not well suited for power magnetics applications wherein operating temperatures frequently exceed 100°C.

EP-A- 095 831 discloses amorphous metal alloys consisting of 4-10% boron, 14-17% silicon and 73-80% iron, by atomic percentages and incidental impurities. These alloys evidence high exciting power (e.g. of the order of 3-5 VA/kg at 60 Hz and 1.4 T) and are not well suited for power magnetics appliations wherein low exciting power is required.

EP-A- 095 803 discloses amorphous metal alloys consisting of 6-10% boron, 14-17% silicon and 1-4% chromium, by atomic percentages, no more than incidental impurities and the balance iron. These chromium containing alloys have relatively low intrinsic saturation induction and relatively low curie temperature, and are unsuitable for elevated temperature, high induction applications.

US-A- 4 437 907 discloses amorphous metal alloys composed of 8-19% silicon, 6-13% boron 0-3.5 carbon and 74-80% iron, by atomic percentage with incidental impurities. These alloys evidence low crystallization temperatures (e.g. less than 515°C) and, hence, are not well suited for power magnetics applications.

EP-A- 0 058 269 discloses amorphous metal alloys consisting essentially of 12 to 16% boron, 5 to 10% silicon and 77 to 80% iron, by atom percent, with no more than incidental impurities. No disclosure is contained therein concerning alloys which exhibit, in combination, enhanced induction at elevated temperatures term thermal stability and low exciting power.

At the time that the amorphous alloys described above were discovered, they evidenced magnetic properties that were superior to then known polycrystalline alloys. Nevertheless, new applications requiring improved magnetic properties at elevated temperatures and higher thermal stability have necessitated efforts to develop additional alloy compositions.

In accordance with the present invention, there is provided a metal alloy which is at least 90 % amorphous having the formula FeₐSi_{b}B_{c} wherein "a", "b" and "c" are atomic percentages ranging from 79.4 to 79.8, 6 to 8 and 12 to 14, respectively, with the proviso that the sum of "a", "b", "c" and impurities equals 100, said alloy having a power loss of less than about 0.3 W/kg, measured at 60 Hz and 1.4 T at 100 °C, a saturation induction value of at least 1.5 T at 100 °C under a drive field of 8000 A/m, and an exciting power less than 1 VA/kg, measured at 60 Hz and 1.4 T, at 100 °C.

The alloys are fabricated by a known process which comprises forming a melt of the desired composition and quenching at a rate of at least about 10⁵ °C/sec by casting molten alloy onto a repidly rotating chill wheel.

In addition, the invention provides a method of enhancing the magnetic properties of a metal alloy which is at least 90 % amorphous having the formula FeₐSi_{b}B_{c} wherein "a", "b" and "c" are atomic percentages ranging from 79.4 to 79.8, 6 to 8 and 12 to 14, respectively, with the proviso that the sum of "a", "b", "c" and impurities equals 100, which method comprises the step of:
heating said alloy to a temperature in the range of about 340°C to 440°C;
cooling said alloy at a rate of about 1°C/min. to 10°C/min.;
and
applying a magnetic field to said alloy during said heating and cooling, wherein the alloy has a power loss of less than about 0.3 W/kg, measured at 60 Hz and 1.4 T at 100°C, a saturation induction value of at least 1.5 T at 100°C under a drive field of 8000 A/m, and an exciting power less than 1 VA/kg measured at 60 Hz and 1.4 T, at 100°C.

Further, the invention provides a core for use in an electromagnetic device; such core comprising a metal alloy as defined above.

The alloys of this invention exhibit improved AC magnetic properties at temperatures ranging from about 100 to 150°C. As a result, the alloys are particularly suited for use in power transformers, aircraft transformers, current transformers, high frequency transformers (e.g. transformers having operating frequencies ranging from about 400 Hz to 100 kHz), switch cores, high gain magnetic amplifiers and low frequency inverters.

The invention will be more fully understood and further advantages will become apparent when reference is made to the following detailed description and the accompanying drawings in which:
Fig. 1 is graph comparing thermal stability (i.e., percent change in 1.4 T/60 Hz exciting power as a function of iron content) for alloys within and outside the scope of the invention; and
Fig. 2 is a graph comparing saturation induction (i.e., induction measured at 8000 A/m and 100°C) as a function of iron content for alloys within and outside the scope of the invention.

The new amorphous Fe-Si-B alloy, in accordance with the invention exhibits enhanced AC magnetic properties at elevated temperatures. The improved magnetic properties are evidenced by high magnetization, low core loss and stable at temperatures ranging from about 100 to 150 °C. A preferred composition within the foregoing ranges consists of 79.4 to 79.7, especially of 79.5 atom percent iron, 13 atom percent boron, the balance being silicon. Another preferred composition contains 6.2 to 7.7 atom percent Si and 12.5 to 14 atom percent B.

The alloys of the invention are at least about 90% amorphous and preferably at least about 97% amorphous and most preferably 100% amorphous. Magnetic properties are improved in alloys possessing a greater volume percent of amorphous material. The volume percent of amorphous material is conveniently determined by X-ray diffraction.

The amorphous metal alloys are formed by cooling a melt at a rate of about 10⁵° to 10⁶°C/sec. The purity of all materials is that found in normal commercial practice. A variety of techniques are available for fabricating splat-quenched foils and rapid-quenched continuous ribbons, wire, sheet, etc. Typically, a particular composition is selected, powders or granules of the requisite elements (or of materials that decompose to form the elements, such as ferroboron, ferrosilicon, etc.) in the desired proportions are melted and homogenized, and the molten alloy is rapidly quenched on a chill surface, such as a rotating cylinder.

The most preferred process for fabricating continuous metal strip containing the alloys of the invention is that set forth in US-A- 4 142 571.

This patent, which is incorporated herein by reference thereto, sets forth a method of forming a continuous metal strip by depositing molten metal onto the surface of a moving chill body. The method comprises the steps of (a) moving the surface of a chill body in a longitudinal direction at a constant predetermined velocity of from about 100 to about 2000 meters per minute past the orifice of a slotted nozzle defined by a pair of generally parallel lips located proximate to the surface such that the gap between the lips and the surface is from about 0.03 to about 1 millimeter, the orifice being arranged generally perpendicular to the direction of movement of the chill body, and (b) forcing a stream of molten metal through the orifice of the nozzle into contact with the surface of the moving chill body to permit the metal to solidify thereon to form a continuous strip. Preferably, the nozzle slot has a width of from about 0.34 to 1 millimeter, the first lip has a width at least equal to the width of the slot and the second lip has a width of from about 1.5 to 3 times the width of the slot amorphous metal strip produced in accordance with the Narasimhan process has a width of at least about 7 millimeters, preferably at least about 1 centimeter and, more preferably yet, a width of at least about 3 centimeters. The strip is at least 0.02 millimeter thick but may be as thick as about 0.14 millimeter, or thicker, depending on the melting point, solidification and crystallization characteristics of the alloy employed.

The alloys of the present invention have an improved processability as compared to other iron-based metallic glasses, since the subject alloys demonstrate a minimized melting point and maximized undercooling.

The magnetic properties of the subject alloys can be enhanced by annealing the alloys. The method of annealing generally comprises heating the alloy to a temperature sufficient to achieve stress relief but less than that required to initiate crystallization, cooling the alloy, and applying a magnetic field to the alloy during the heating and cooling. Generally, a temperature range of about 340°C to 440°C is employed during heating. A rate of cooling range of about 0.5°C/min. to 75°C/min. is employed, with a rate of about 1°C/min. to 16°C/min. being preferred.

As discussed above, the alloys of the present invention exhibit improved magnetic properties (particularly higher saturation induction) that are stable at temperatures ranging from about 100 to about 150°C, rather than a maximum of 125°C as evidenced by prior art alloys. The increased temperature stability of the present alloys allows utilization thereof in high temperature applications, such as cores in transformers for distributing electrical power to residential and commercial consumers.

More specifically, for the Fe-B-Si compositions disclosed hereinabove, superior loss and exciting power characteristics can be achieved by proper selection of annealing conditions. Apart from loss and exiting power characteristics, two other criteria, namely, saturation induction at elevated temperature and thermal stability are crucial to and should be optimized for power magnetics applications.

Saturation induction at elevated temperature can be approximated by measuring B 8000 A/m at 100°C. Figure 2 is a graph comprising saturation induction (i.e., induction measured at B 8000 A/m and 100°C) as a function of iron content for Fe-B-Si containing alloys within and outside the scope of the invention. As illustrated by Figure 2, the saturation induction at 100°C for alloys containing above about 79.4 atom percent iron is about 1% higher than that of alloys having iron content less than 79.4. From the standpoint of loss evaluation, this gain in operating induction at elevated temperature decreases the size of the transformer and significantly enhances the intrinsic value of the amorphous alloys as a power magnetic core material.

The long range thermal stability can be approximated by accelerated aging as discussed by Datta et al. in the Proceedings of a Symposium on "Chemistry and Physics of Rapidly Solidified Materials" held at St. Louis, Missouri, October 26-27, 1982 by the Metallurgical Society of AIME. Acceleration aging consists of estimating change in important soft magnetic properties (e.g., % change in VA at 1.4 T/60 Hz) of prototype cores exposed to temperatures higher than normal operating temperatures and extrapolating the change in properties to operating temperatures. Figure 1 is a graph comparing accelerated aging (i.e., thermal stability) behavior (i.e., percent changes 1.4 T 60 Hz exciting power as a function of iron content) for Fe-B-Si containing alloys within and outside the scope of the invention. Aging was conducted at 240°C for 2200 hrs. As illustrated by Figure 1, alloys containing above about 79.8 atom percent iron experienced a substantial increase in exciting power (i.e., were aged significantly). Advantageously, each of the elevated temperature saturation induction and thermal stability were simultaneously optimized for alloys within the scope of the invention having iron content ranging from above about 79.4 to 79.8.

When cores comprising the subject alloys are utilized in electromagnetic devices, such as transformers, they evidence exceedingly high magnetization, low core loss and low volt-ampere demand, thus resulting in more efficient operation of the electromagnetic device. The loss of energy in a magnetic core as the result of eddy currents, which circulate through the core, results in the dissipation of energy in the form of heat. Cores made from the subject alloys require less electrical energy for operation and produce less heat. In applications where cooling apparatus is required to cool the transformer cores, such as transformers in aircraft and large power transformers, an additional savings is realized since less cooling apparatus is required to remove the smaller amount of heat generated by cores made from the subject alloys. In addition, the exceedingly high magnetization and high efficiency of cores made from the subject alloys result in cores of reduced weight for a given capacity rating.

The following examples are presented to provide a more complete understanding of the invention.

### EXAMPLES

Toroidal test samples were prepared by winding approximately 0.030 kg of 0.0254 m wide alloy ribbon of various compositions containing iron, silicon and boron on a steatite core having inside and outside diameters of 0.0397 m and 0.0445 m, respectively. One hundred and fifty turns of high temperature magnetic wire were wound on the toroid to provide a D.C. circumferential field of 795.8 ampere/meter for annealing purposes. The samples were annealed in an inert gas atmosphere for 2 hours at a temperature ranging from 340°C to 440°C with the 795.8 A/m field applied during heating and cooling to determine the optimum field annealing conditions for each composition. The optimum field annealing condition for each composition is that at which the exciting power of the core is lowest. The samples were cooled at a rate of approximately 10°C/min.

The AC magnetic properties, i.e., power loss (watts/kilogram) and exciting power (volt-amperes/ kilogram), of the samples were measured at a frequency of 60 Hz and a magnetic intensity of 1.4 Tesla by the sine-flux method.

Field annealed AC magnetic values for a variety of alloy compositions that are within the scope of the present invention are shown in Table I.

For comparison, the compositions of some amorphous metal alloys lying outside the scope of the invention and their field annealed AC measurements are listed in Table II. These alloys, in contrast to those within the scope of the present invention, have higher core loss and higher volt-ampere demand at room temperature and at 100°C.

To illustrate the improved saturation induction of alloy compositions of the present invention at elevated temperatures, each of samples 1-6 from Table I was further tested by exciting each sample with an 8000 A/m drive field at 100°C. The improved saturation induction of the alloys thus tested is shown in Table III.

For comparison, the compositions of some amorphous metal alloys falling outside the scope of the invention and their saturation induction measurements at 8000 A/m drive field and 100°C are set forth in Table IV.

## Claims

1. A metal alloy which is at least 90 % amorphous having the formula FeₐSi_{b}B_{c} wherein "a", "b" and "c" are atomic percentages ranging from 79.4 to 79.8, 6 to 8 and 12 to 14, respectively, with the proviso that the sum of "a", "b", "c" and impurities equals 100, said alloy having a power loss of less than about 0.3 W/kg, measured at 60 Hz and 1.4 T at 100 °C, a saturation induction value of at least 1.5 T at 100 °C under a drive field of 8000 A/m, and an exciting power less than 1 VA/kg, measured at 60 Hz and 1.4 T, at 100 °C.

2. The metal alloy as recited in claim 1, wherein "a" and "c" are 79.4 to 79.7 and 13 respectively, the balance being silicon.

3. The metal alloy as recited in claim 1 wherein "b" ranges from 6.2 to 7.7 and wherein "c" ranges from 12.5 to 14.

4. A method of enhancing the magnetic properties of a metal alloy which is at least 90 % amorphous having the formula FeₐSi_{b}B_{c} wherein "a", "b" and "c" are atomic percentages ranging from 79.4 to 79.8, 6 to 8 and 12 to 14, respectively, with the proviso that the sum of "a", "b", "c" and impurities equals 100, which method comprises the step of:
heating said alloy to a temperature in the range of about 340 °C to 440 °C;
cooling said alloy at a rate of about 1 °C/min to 10 °C/min and
applying a magnetic field to said alloy during said heating and cooling, wherein the alloy has a power loss of less than about 0.3 W/kg, measured at 60 Hz and 1.4 T at 100 °C, a saturation induction value of at least 1.5 T at 100 °C under a drive field of 8000 A/m, and an exciting power less than 1 VA/kg measured at 60 Hz and 1.4 T, at 100 °C.

5. A core for an electromagnetic device comprising a metal alloy which is at least 90 % amorphous having the formula FeₐSi_{b}B_{c} wherein "a", "b", "c" and impurities are atomic percentages ranging from 79.4 to 79.8, 6 to 8 and 12 to 14, respectively, with the proviso that the sum of "a", "b" and "c" and impurities equals 100, said alloy having the form of ribbon and having been annealed, said alloy exhibiting a power loss of less than about 0.3 W/kg, measured at 600 Hz and 1.4 T, a saturation induction of at least 1.50 T at 100 °C under a drive field of 8000 A/m, and an exciting power less than 1 VA/kg, measured at 60 Hz and 1.4 T, at 100 °C.

## Revendications

1. Alliage métallique amorphe au moins à 90% et ayant pour formule FeₐSi_{b}B_{c}, où "a", "b" et "c" sont des pourcentages atomiques allant respectivement de 79,4 à 79,8, de 6 à 8 et de 12 à 14, avec comme condition que la somme de "a", "b", "c" et celle des impuretés soit égale à 100, ledit alliage présentant une perte de puissance inférieure à environ 0,3 W/kg mesurée à 60 Hz, 1,4 T et 100°C, une valeur de l'induction de saturation d'au moins 1,5 T à 100°C sous un champ d'excitation de 8000 A/m et une puissance d'excitation inférieure à 1 VA/kg mesurée à 60 Hz, 1,4 T et 100°C.

2. Alliage métallique comme décrit dans la revendication 1, où "a" et "c" sont égaux respectivement à 79,4 - 79,7 et à 13, le restant étant du silicium.

3. Alliage métallique comme décrit dans la revendication 1, où "b" se situe entre 6,2 et 7,7 et où "c" se situe entre 12,5 et 14.

4. Méthode pour améliorer les propriétés magnétiques d'un alliage métallique amorphe au moins à 90% et ayant pour formule FeₐSi_{b}B_{c}, où "a", "b" et "c" sont des pourcentages atomiques allant respectivement de 79,4 à 79,8, de 6 à 8 et de 12 à 14, avec comme condition que que la somme de "a", "b", "c" et celle des impuretés soit égale à 100, laquelle méthode comprend les étapes consistant à :
chauffer ledit alliage à une température dans la gamme allant environ de 340°C à 440°C;
refroidir ledit alliage à une vitesse d'environ 1°C/min à 10°C/min; et à
appliquer un champ magnétique audit alliage durant lesdits chauffage et refroidissement, où l'alliage présente une perte de puissance inférieure à environ 0,3 W/kg mesurée à 60 Hz, 1,4 T et 100°C, une valeur de l'induction de saturation d'au moins 1,5 T à 100°C sous un champ d'excitation de 8000 A/m et une puissance d'excitation inférieure à 1 VA/k mesurée à 60 Hz, 1,4 T et 100°C g.

5. Noyau pour un dispositif électromagnétique comprenant un alliage métallique amorphe au moins à 90% et ayant pour formule FeₐSi_{b}B_{c}, où "a", "b" et "c" et les impuretés sont des pourcentages atomiques allant respectivement de 79,4 à 79,8, de 6 à 8 et de 12 à 14, avec comme condition que la somme de "a", "b", "c" et celle des impuretés soit égale à 100, ledit alliage ayant la forme d'un ruban et ayant subi une recuisson, ledit alliage présentant une perte de puissance inférieure à environ 0,3 W/kg mesurée à 600 Hz et 1,4 T, une induction de saturation d'au moins 1,5 T à 100°C sous un champ d'excitation de 8000 A/m et une puissance d'excitation inférieure à 1 VA/kg mesurée à 60 Hz, 1,4 T et 100°C

## Patentansprüche

1. Metallegierung, die zu wenigstens 90 % amorph ist und die Formel FeₐSi_{b}B_{c} hat, worin "a", "b" und "c" Atomprozentsätze im Bereich von 79,4 bis 79,8, 6 bis 8 bzw. 12 bis 14 sind, wobei die Summe von "a", "b", "c" und Verunreinigungen 100 ist und wobei diese Legierung eine Verlustleistung von weniger als etwa 0,3 W/kg, gemessen bei 60 Hz und 1,4 T bei 100 °C, einen Sättigungsinduktionswert von wenigstens 1,5 T bei 100 °CG unter einem Antriebsfeld von 8000 A/m und eine Erregerkraft von weniger als 1 VA/kg, gemessen bei 60 Hz und 1,4 T bei 100 °C, hat.

2. Metallegierung nach Anspruch 1, worin "a" und "c" 79,4 bis 79,7 bzw. 13 sind, wobei der Rest Sillicium ist.

3. Metallegierung nach Anspruch 1, worin "b" im Bereich von 6,2 bis 7,7 liegt und worin "c" im Bereich von 12,5 bis 14 liegt.

4. Verfahren zur Verbesserung der magnetischen Eigenschaften einer Metallegierung, die zu wenigstens 90 % amorph ist und die Formel FeₐSi_{b}B_{c} hat, worin "a", "b" und "c" Atomprozentsätze im Bereich von 79,4 bis 79,8, 6 bis 8 bzw. 12 bis 14 sind und wobei die Summe von "a", "b", "c" und Verunreinigungen 100 ist, mit der Stufe, in der man
die Legierung auf eine Temperatur im Bereich von etwa 340 °C bis 440 °C erhitzt,
die Legierung mit einer Geschwindigkeit von etwa 1 °C/min bis 10 °C/min abkühlt und
während des Erhitzens und Abkühlens ein Magnetfeld an diese Legierung anlegt, wobei die Legierung eine Vertustleistung von weniger als etwa 0,3 W/kg, gemessen bei 60 Hz und 1,4 T bei 100 °C, einen Sättigungsinduktionswert von wenigstens 1,5 T bei 100 °C unter einem Antriebsfeld von 8000 A/m und eine Erregerkraft von weniger als 1 VA/kg, gemessen bei 60 Hz und 1,4 T bei 100 °C, hat.

5. Kern für eine elektromagnetische Vorrichtung mit einer Metallegierung, die zu wenigstens Atomprozente im Bereich von 79,4 bis 79,8, 6 bis 8 bzw. 12 bis 14 sind und wobei die Summe von "a", "b", "c" und Verunreinigungen 100 ist, wobei diese Legierung die Form eines Bandes hat und geglüht wurde und die Legierung eine Verlustleistung von weniger als etwa 0,3 W/kg, gemessen bei 600 Hz und 1,4 T, eine Sättigungsinduktion von wenigstens 1,50 T bei 100 °C unter einem Antriebsfeld von 8000 A/m und eine Erregerkraft von weniger als 1 VA/kg, gemessen bei 60 Hz und 1,4 T bei 100 °C, hat.
